

Feb. 2, 1971

H. HEINEN

3,560,271

## NITRIDING METHOD

Filed May 16, 1968

Fig. 1



Fig. 2 21



Fig.



Fig. 3



Inventor:  
Hans Heinen  
By Michael S. Stretton  
Attorney

1

3,560,271

## NITRIDING METHOD

Hans Heinen, Meinerzhagen, Germany, assignor to Otto Fuchs, Meinerzhagen, Germany  
Filed May 16, 1968, Ser. No. 730,216  
Claims priority, application Germany, May 17, 1967,  
F 52,437  
Int. Cl. C23c 9/14; C21d 1/74  
U.S. Cl. 148—15.5 7 Claims

### ABSTRACT OF THE DISCLOSURE

Metallic work pieces, particularly alloyed steel work pieces are nitrided at temperatures above 500° C. and are then conveyed into a pressure vessel at such speed that during conveying of the work piece the temperature thereof will drop relatively little, not more than 100° C. and preferably so that the workpiece when introduced into the pressure vessel still has a temperature of at least about 500° C. Promptly after introduction of the hot work piece, the pressure vessel is evacuated and the hot work piece is allowed to cool by heat radiation while being located in the evacuated pressure vessel. Cooling in the above described manner will improve the quality of the nitrided work piece.

### BACKGROUND OF THE INVENTION

The present invention is concerned with the nitriding of metallic work pieces, particularly work pieces of highly alloyed metals and primarily work pieces of alloyed steel, whereby the steel may be alloyed, for instance, with one or more of the metals nickel, manganese, chromium, molybdenum, vanadium and tungsten.

Such alloyed steels are used for tools and also for machine parts which must withstand sliding contact, such as crankshafts, pistons and cylinders in which pistons are to move. Such products are progressively more sensitive with respect to crack formation the higher the proportion of alloy constituents therein. For this reason, as will be discussed further below, the advantages of the present invention are particularly significant with respect to tools and work pieces of highly alloyed metals. However, the invention is not necessary limited to the treatment of highly alloyed steel. For instance, the present invention is also highly advantageous in connection with the nitriding of stellite, i.e. an alloy of predominantly chromium and cobalt.

Nitriding may be carried out in various manners known per se in the art and the present invention is particularly concerned with modifications of the nitriding, particularly the subsequent cooling of the nitrided work piece, in such cases in which the nitriding is carried out in molten nitriding salt mixtures, for instance by the method known as the "Tenifer" method of the firm Degussa, Germany. This method comprises melting a mixture of nitrogen-containing salts and immersing the work pieces which are to be nitrided into the molten salt bath.

This and other conventional nitriding methods permit excellent hardening of alloyed metals, particularly highly alloyed steel, whereby the work pieces also may be formed of sintered metals. Contrary to the conventional cementing methods, such nitriding gives particularly high hardness values; however, the depth or penetration of the thus-formed nitride layer is rather limited, especially in the case of highly alloyed metals even if the nitriding is carried out for prolonged periods of time. The depth of nitriding may reach values of barely hundred microns; however, this depth refers to the depth of diffusion of nitrogen and not to the depth to which actually a nitrogen-containing metal compound such as  $Fe_4N$  is formed.

2

This compound zone generally has a thickness of only about 10–20 microns. The exact composition of the "compound zone" is of no concern here, but it is important to note that there is formed by nitriding a relatively thin "compound zone," much thinner than the zone of diffusion, which compound zone is mainly responsible for the hardness of the treated work piece and may consist for instance of a complex compound of cementite and nitride such as  $Fe_3C \cdot Fe_4N$ . At a greater depth, i.e. within the remaining diffusion zone, nitrogen atoms will be found but not the alloy or compound  $Fe_4N$ .

It is an important feature of nitriding that the above-described "compound zone" is so very thin, i.e. generally has a thickness of only up to about 20 microns.

5 Due to the small cross-sectional dimensions of the hard, outer compound layer or zone formed during the nitriding in molten nitriding salt, the thin hard layer is very critical and cannot be recreated by welding upon additional material the compound zone being a complex combination 10 with nitrogen. Moreover during cooling of the hot nitrided work pieces a considerable risk exists that for the reasons discussed above tension cracks will be formed. Such tension cracks may occur during cooling and also immediately after completion of the hot nitriding, 15 depending on the conditions under which the cooling is carried out, for instance in a water or oil bath.

More moderate cooling by exposure to air cannot be carried out since, as is well known, upon cooling in contact with air damaging surface corrosion phenomena 20 occur.

However, frequently, such cracks are formed only after putting the nitrided work piece, for instance a tool, into operation. For instance, in dies for extrusion presses used for producing profiled light metal building elements which 25 have relatively complicated cross-sectional configurations, considerable stresses will be found, particularly in corner portions of the die profile which even under a low load or after a short period of operation will cause crack formation and thereby render the die unusable.

40 It is thus most desirable to carry out the cooling of the hot nitrided work pieces in a moderate and protective manner; however, up to now no practical and fully satisfactory solution has been found for this problem. Particularly, it is not possible to reduce the undesirable tensions

45 by carrying out the cooling of the freshly nitrided hot work piece by blowing air or hot air against the work piece. This will retard the speed of cooling; however, the salt-holding work piece surfaces tend to react with the oxygen of the air with formation of firmly adhering surface 50 layers consisting essentially of the thus-formed reaction products. Subsequent surface treatment of the cooled work piece is not possible since it would reduce the cross-sectional dimension of the hard compound zone which, as pointed out above, is very small to begin with, and 55 thereby the useful life span of the thus-nitrided and cooled work piece would be at least considerably reduced.

Thus, the problem of cooling the freshly nitrided work pieces which in liquid nitriding salt solutions generally 60 were heated to a temperature of somewhat below 600° C., such as 570° C., represents a very serious problem. The nitrided work pieces are highly sensitive against surface corrosion by reaction with oxygen and against the formation of tension cracks. Particularly if the hard 65 nitrided compound zone at the surface of the work piece is combined with complicated configurations, heat tensions occur as soon as the work piece is taken from the molten salt bath and subjected to cooling. If cooling is carried out sufficiently slowly so as to avoid such heat-caused 70 tensions, then a very harmful corrosion layer will be formed on the surface of the hard compound zone of nitrided metal which corrosion layer can only be removed

with very great difficulties, if at all, for instance if the work piece is of complicated shape as for instance indicated by reference numeral 21 in FIG. 2 of the drawing.

On the other hand, if cooling is carried out at a faster rate so that the corrosion risk is reduced, then the heat tensions will not be equalized or balanced and crack formation or even breaking of the work piece may occur.

Thus, up till now no practically successful method did exist for nitride-hardening of work pieces of certain complicated surface configurations since nearly always cracking of the metal occurred when it was attempted to avoid excessive corrosion of the surface.

It is an object of the present invention to provide a method and device or arrangement which will overcome these difficulties and will result in obtaining cooled nitrided work pieces which are not excessively corroded and in which the interior heat tensions are nearly completely equalized.

Furthermore, even if in conventional manner the hot nitrided work pieces were cooled by immersion in a suitable cooling liquid and thus excessive corrosion of the surface by contact with the oxygen of the air has been avoided, nevertheless, lapping or wet-honing is necessary and this cleaning of the surface generally has to be carried out in a series of steps and will not be effective with respect to surface portions which are inaccessible or only difficultly accessible.

However, the removal of corrosion layers which are formed even upon cooling in liquid media (thereby risking crack formation) is practically impossible with respect to, for instance, the interior surface portions of an extrusion die. The removal of such corrosion layers, however, is necessary and important if upon operation of the die in an extrusion device, extruded bodies of the desired smooth surface configuration are to be obtained.

All these measures do not only require substantial labor but are also connected with the risk that the hard nitrided surface layer of the respective work piece will be damaged thereby and thus would have to be further worked. Frequently, hardened work pieces with damaged surface layers which can no longer be reconditioned represent a valueless or practically valueless waste material.

It would be possible to consider prevention of formation of corrosion layers by maintaining the work pieces after hot nitriding and until they are cooled to, for instance, room temperature, in an inert atmosphere such as a nitrogen atmosphere. However, the costs and difficulties in controlling the individual steps of the process if the same has to be carried out in a nitrogen or the like atmosphere have been found to be practically insurmountable so that the cooling in a nitrogen atmosphere in which the hot work piece would have to be maintained upon removal from the nitriding bath until it is sufficiently cooled, did not meet with practical success.

The same holds true for operating in a vacuum which possibly could be done under laboratory conditions, but would not lend itself to industrial operations, considering the weight of the work pieces, the necessity of maintaining the molten nitriding salt bath and the conveying devices for removing the work piece therefrom as well as the resting place for the work piece during cooling thereof, under such reduced pressure and thereby in a substantially oxygen-free atmosphere.

It is therefore an object of the present invention to overcome the above-discussed difficulties and disadvantages, to simplify the cooling of hot nitrided work pieces, particularly work pieces which were nitrided by immersion in a molten bath of nitriding salts, so that even in the case of work pieces of complicated surface configuration tension-crack formation is substantially avoided and at the same time the formation of harmful surface layers such as the above-described corrosion layers or the like will be substantially or fully eliminated so that subsequent working of the surface of the cooled nitrided work piece by lapping or other cleaning methods can be reduced to a minimum.

#### SUMMARY OF THE INVENTION

According to the present invention, metallic work pieces are nitrided by subjecting the work piece to nitriding at a nitriding temperature which is significantly above about 500° C., generally somewhat below 600° C. and frequency about 570° C. The thus-nitrided hot work piece is then conveyed through the ambient atmosphere into an evacuable zone at such speed that during passage through the ambient atmosphere the temperature of the hot nitrided work piece will drop only slightly, generally less than about 100° C. and preferably not below about 500° C. Immediately after the work piece has been placed into the evacuable zone, the latter is evacuated to a residual pressure of up to about 20 mm. of mercury, preferably to between 2 and 20 mm. mercury, or up to 2 mm. mercury, and the still hot work piece, which has been introduced into the evacuable zone at a temperature preferably above or not lower than about 500° C., will then be allowed to cool by heat radiation while located in the thus-evacuated zone.

The metallic work piece may be and frequently is formed of highly alloyed steel and the cooling in the evacuated zone may be continued until the work piece has reached room temperature, but generally it will suffice to continue cooling by heat radiation of the work piece located in the evacuated zone until the temperature of the work piece has been lowered to about 150° C., since at a temperature of about 150° C., practically no reaction between the surface layer of the work piece and the oxygen of ambient air would occur.

The evacuated zone preferably is represented by the interior of a pressure vessel into which the work piece is introduced, whereupon the pressure vessel is closed and evacuated.

Since the heat radiation emanating from the work piece would eventually lead to heating of the wall of the pressure vessel and thus to causing a counter-current heat radiation from the walls of the pressure vessel towards the work piece, thereby possibly unduly retarding the cooling process, it is frequently preferred to cool the walls of the pressure vessel, or portions of the walls thereof in conventional manner, for instance by spraying the outside of the pressure vessel with water or arranging cooling coils thereon of any other of the many methods known for this purpose to those skilled in the art.

In any event, the heat withdrawal from the hot work piece takes place by heat radiation therefrom while the work piece is located in the evacuated interior of the pressure vessel.

The present invention is also concerned with an arrangement for carrying out the above described method which arrangement comprises a nitriding furnace or vessel in which a molten bath of nitriding salts is maintained, the above-described pressure vessel, suitable conduits and a vacuum pump or the like for evacuating the pressure vessel, conveying apparatus for lifting the nitrided hot work piece from the molten salt bath and introducing it into the pressure vessel, and electronic control arrangements for actuating the conveying arrangement, the vacuum pump or the like, and possibly also for opening and closing the lid of the pressure vessel in accordance with a preset schedule which may be made dependent on readings of time and temperature.

Since in many cases the length of the cooling period may exceed the time required for nitriding the work piece, it is also within the scope of the present invention to provide an arrangement in which a plurality of pressure vessels is combined with a lesser number, or one, nitriding furnace or molten bath of nitriding salts so that the nitriding bath or furnace may be used to its full capacity by successively feeding the hot nitrided work pieces into different ones of the series of pressure vessels arranged in the vicinity of the nitriding furnace. The conveying of the hot nitrided work pieces to specific ones of the series of pressure vessels also may be electronically

controlled in a manner which, *per se*, will be apparent to those skilled in the art.

The novel features which are considered as characteristic for the invention are set forth in particular in the appended claims. The invention itself, however, both as to its construction and its method of operation, together with additional objects and advantages thereof, will be best understood from the following description of specific embodiments when read in connection with the accompanying drawing.

#### BRIEF DESCRIPTION OF THE DRAWING

FIG. 1 is a schematic, elevational, perspective view of a complete nitriding arrangement in accordance with the present invention; and

FIG. 2-4 are illustrations, on a scale larger than that of FIG. 1, of specific work pieces which may be advantageously nitrided in accordance with the present invention.

#### DESCRIPTION OF THE PREFERRED EMBODIMENTS

In connection with the solution of the above-discussed problems in accordance with the present invention, two basic concepts should be considered.

With respect to the danger of formation of tension cracks, it is quite clear that this danger depends on the type and manner of the cooling process to which the hot, freshly nitrided work pieces are exposed, whereby generally heat is given up by the work pieces by heat conduction and convection. Heat loss by radiation may be disregarded inasmuch as, in accordance with Boltzmann's Law, the radiation of heat is proportional to the fourth power of the respective temperature differential and thus will be important only during the initial cooling of the still rather hot work piece, and it is well known that in this temperature range, *i.e.* while the work piece is still at a temperature relatively close to the nitriding temperature, heat cracks generally do not occur.

Consequently, the withdrawal of heat and thus the cooling of the work piece by radiation would be particularly desirable and even more so during progressive cooling since heat radiation emanates essentially in radial direction, *i.e.* eccentrically relative to the work piece and, consequently, the interior configuration, particularly interior surfaces of the work piece play only a relatively unimportant role.

Work pieces with complicated inner surfaces, such as extrusion dies having inner surfaces which in part are outwardly flaring, would be severely endangered by cooling in a medium such as gas or liquid which would directly contact such inner surface portions. On the other hand, the zone of these inner surface portions would participate only very slightly or practically not at all in the initial heat withdrawal by radiation since in this case, between closely adjacent inner surface portions, even desirable heat or temperature equalizations would occur and consequently absorption or reflection of heat rays would to a considerably extent compensate each other. Thus, a work piece with such complicated interior surface configurations would radiate approximately the same amount of heat into the surrounding space as a simple solid metal body of similar outer shape and surface. The speed of cooling or the period of time required for cooling of work pieces of equal mass, which by itself is not of particular importance, will be nearly the same irrespective of differences in the surface configuration, particularly the configuration of inner surfaces, of the work pieces.

The second concept which is to be considered in connection with the present invention, is concerned with the formation of undesirable surface or corrosion layers. The formation of surface layers takes place not so much at the point or moment of withdrawal of the work piece from the molten salt bath and its exposure to the ambient atmosphere but only somewhat later, namely after the oxygen of the air had time to diffuse through the salt

layer adhering to the surface of the work piece and thus to come into direct contact with the metal surface of the work piece. It has been found that harmful surface layers are formed by the effect of contact with the ambient atmosphere only after the work piece had been removed from the molten salt bath for a certain length of time.

It thus has been surprisingly found in accordance with the present invention that it is possible to expose the work piece immediately after removal of the same from the molten salt bath, for a limited period of time, provided that the contact between the work piece (with a salt layer adhering thereto) and the ambient atmosphere is effectively interrupted after a relatively short period of time.

15 It would seem that these two concepts cannot be co-ordinated since the desired retardation of cooling for the purpose of avoiding tension-crack formation necessarily requires maintenance of relatively high temperatures and thus greater reactivity for prolonged periods of time, particularly since the use of inert gases as cooling fluid does not represent an economically feasible solution of this problem.

However, in order to approach the theoretically desired or ideal conditions and to obtain the technical advantages 25 of cooling of the work piece by heat radiation at reduced surrounding pressure as well as to avoid chemical surface reactions by substantially exclusion of oxygen and moisture in a relatively simple and economical manner, it is proposed according to the present invention to convey the 30 work pieces, as they are withdrawn from the nitriding molten salt bath, without any control of temperature or chemical reactions, but without substantial delay, through the ambient atmosphere into a closable pressure vessel, and thereafter to evacuate the pressure vessel to a residual pressure of at most about 20 and preferably about 25 2 mm. mercury, whereupon cooling of the work piece will take place by heat radiation while the work piece is located in the evacuated vessel.

Surprisingly, it has been found by proceeding as outlined above, that the cooling by convection which takes place during the relatively short period of time during which the work piece is transported in contact with the ambient air from the nitriding vessel to the pressure vessel will not increase the risk of the formation of tension cracks as compared with laboratory experiments in which 45 the work piece was maintained in a partial vacuum from the moment of leaving the nitriding bath until sufficiently cooled.

By proceeding in this manner discards were no longer 50 obtained, *i.e.* work pieces which were unusable due to formation of tension cracks, and thus it became possible to nitride work pieces of very complicated surface configurations, particularly inner surface portions, in a much more reliable and effective manner than was believed possible up to now.

According to the present invention, the work pieces have to be conveyed from the hot salt bath into the pressure vessel. It is desired to carry out this conveying as quickly as possible. However, no harm is done if during such 60 conveying the work piece is cooled by up to about 100° C. At the beginning of the conveying, the surface of the work piece is still covered by salt and, consequently, there is little risk of corrosion. Furthermore, obviously, at the beginning of the cooling no interior heat tensions 65 will occur and this also is essential in accordance with the present invention.

Consequently, it is possible to expose the work piece for a limited period of time during the conveying from the molten salt bath to the pressure vessel to the influence 70 of the ambient atmosphere. The exact length of time for which the work piece may be exposed to the ambient atmosphere prior to being subjected to reduced pressure in the pressure vessel, and the extent to which the work piece may be cooled during such transfer and prior to being exposed to the reduced pressure, will depend on

the size and mass of the work piece and to some extent on the manner in which the entire nitriding facilities are arranged. Smaller work pieces may be more quickly conveyed into the pressure vessel and, nevertheless, the temperature of such smaller work pieces may drop by about 100° C. prior to being exposed to reduced pressure.

On the other hand, large and heavy work pieces, for instance crankshafts, cannot be conveyed with such speed and thus it may take up to about one minute or so from the withdrawing of the work piece from the molten salt bath until the work piece is subjected to the pressure reduction. However, due to the greater mass of such larger work piece, the cooling during the relatively prolonged period of time, namely about one minute, may be as little as 50° C.

The preferred temperature of molten salt nitriding baths is about 570° C. and it is desirable that the temperature of the work piece upon being introduced into the pressure vessel, i.e. immediately prior to evacuation of the pressure vessel, should still be somewhat above 500° C. To expose the work piece to the reduced pressure while the temperature thereof is still above 500° C. is particularly important in the case of complicated surface configurations.

On the other hand, a relatively simple work piece such as that shown in FIG. 2 and formed with a simple central bore instead of the rather involved configuration of the aperture indicated by reference numeral 21, possibly may be completely cooled while exposed to the ambient atmosphere. However, in such case the work piece would obtain a very rough surface due to the above-discussed chemical reactions which would take place upon such prolonged exposure during cooling to the influence of the oxygen of the ambient atmosphere and it would be most expensive and difficult to subsequently convert such surface into the desired smooth surface.

Surprisingly, it has been found that by proceeding in accordance with the present invention the surface of the cooled work piece remains smooth and substantially free of corrosion or undesirable surface layers. It had been expected that due to the reduced pressure to which the work piece is exposed within a few minutes after being removed from the nitriding bath, the surface conditions of the work piece would be improved.

However, it was still surprising to find that even after completion of the retarded cooling in the evacuated pressure vessel, work pieces, which, for instance, had been retained in the evacuated pressure vessel for about five hours, had a perfectly smooth surface which, after rinsing off of residual salt, in many cases did not require any further working. This seems to be proof of the contention that during the initial short exposure of the hot work piece to the ambient atmosphere the then still present salt layer prevented any significant surface corrosion.

The method of the present invention has been successfully carried out with respect to work pieces of greatly varying configurations and sizes.

Thus, the theoretically achievable advantages of the prohibitively expensive complete vacuum treatment (i.e. vacuum treatment from the moment of withdrawal from the molten salt bath until cooling to a sufficiently low temperature) may be achieved in an extremely simple and economical manner by proceeding in accordance with the present invention which requires only the evacuation of a pressure vessel and not the evacuation of the entire working area, i.e. the entire path along which the work piece must move from withdrawal from the salt bath to being placed at rest in the location where cooling is completed.

It is a further advantage of the present invention that generally no further treatment of the work pieces is required, not only for removing corrosion layers and the like, but also that high gloss polishing of the work piece surface can be carried out in a much more simple manner than was heretofore possible and it is note-

worthy in this connection that the surface of the cooled work piece will have the same dimensions as the freshly nitrided work piece and the hard nitrided outer zone will not be damaged since polishing can be carried out substantially without the removal of material.

5 Additionally, the method of the present invention lends itself excellently to substantial automation and electronic control whereas conventional methods of this type required substantial skilled labor for controlling the cooling process.

10 The work pieces will cool in the evacuated pressure vessel at a rate depending on the mass of the respective work piece whereas the shape of the work piece will be of relatively insignificant importance with respect to the 15 cooling speed in accordance with the present invention. Thus, no special measures have to be taken in order to find out in any given case the most advantageous cooling rate which will avoid the formation of tension cracks.

20 Apart from substantially completely eliminating waste due to crack formation, and substantial reduction of corrosion, the labor costs of the process are substantially lower than that of conventional processes since not only the nitriding in the molten salt bath, but also the cooling 25 of the hardened work piece can be easily and reliably controlled in an automatic manner.

25 Although completely different conditions prevail in the nitriding of work pieces of different alloy composition, different mass and different shapes, no complications arise when proceeding in accordance with the present invention, and the work pieces may be nitrided for the desired length of time and then cooled, which up till now in the case of certain work pieces of particularly complicated configurations could not be successfully accomplished due to corrosion layers and crack formation. Once the required time for nitriding has been determined and the time for cooling by radiation which depends primarily on the mass of the work piece, it is easily possible to automate the process or to subject it to electronic 40 controls. For instance, a switching drum or cam arrangement may be used for controlling all required time intervals. The requirements for skilled labor in carrying out the process of the present invention are thus greatly reduced.

45 The easy control and possible automation of the process of the present invention also facilitates the scheduling of the process since work intermissions do no longer pose a problem. For instance, nitriding in the salt bath may be carried out up to the lunch break or up to the end of the working week and the cooling of the nitrided work 50 pieces in the evacuated pressure vessels will then proceed during the break, week-end or the like, without requiring supervision.

55 While the present invention has been primarily described in connection with salt bath nitriding, it may also be used for the cooling of work pieces which were subjected to nitriding in a hot nitrogen atmosphere, whereby it will not be necessary to subject the nitrogen atmosphere to cooling.

In either case, the apparatus requirements are very 60 limited, particularly since an oil pump for evacuating the pressure vessel may be electronically controlled so as to stop operation when a desired minimum pressure of, for instance, 10 mm. mercury has been reached and, furthermore, one oil pump may serve for the evacuation 65 of a plurality of pressure vessels.

70 By utilizing packings of synthetic material which per se are known to those skilled in the art for achieving an hermetic seal between the lid and the body of the pressure vessel, it is possible to maintain the initially obtained degree of vacuum for prolonged periods of time which suffice for the cooling of the hardened work piece, particularly since temperatures as high as about 150° C. are harmless and thus, the work piece may be exposed to ambient temperature when it has been cooled to about 75 150° C.

Referring now to the drawing and particularly to FIG. 1, it will be seen that the arrangement according to the present invention comprises a molten salt bath furnace 1 of conventional construction with the required auxiliary devices, a conveying device 2 and a pressure vessel 3 which is connected with an electrically operated vacuum pump 4.

Salt bath furnace 1 contains the molten salt mixture of alkali metal cyanate and alkali metal cyanide as required for carrying out nitriding in accordance with the "Tenifer" method.

The conveying device 2 includes a rail on which conveyor elements 5 move in a manner, i.e. at given time intervals, which may be electronically controlled. At the desired moment, work pieces 6 which had been immersed in furnace 1 are lifted with the help of servo motors by reducing the lengths of ropes 7, conveyed to pressure vessel 3 and introduced into the opened pressure vessel by lengthening rope 7.

In the interior of pressure vessel 3, supporting elements (not shown) are provided on which the work pieces 6 will come to rest so that thereby the work pieces will be disconnected from ropes 7. After introduction of the work pieces, lid 10 which is supported by shaft 9, the latter being capable of rotating about its own axis, will be placed in position above opening 11 of pressure vessel 3, and lowered so as to close the pressure vessel. Thereafter, pump 4 is actuated and the interior of pressure vessel 3 is quickly evacuated.

Between the rim of opening 11 of the pressure vessel 3 and lid 10, a packing 12 is arranged, preferably formed of synthetic material commercially available under the name "Teflon." In order to avoid excessive heating of the packing, preferably and in conventional manner water cooling is installed in the side wall and/or top of pressure vessel 3.

Furthermore, a temperature-sensing instrument 13, such as a thermometer, extends inwardly through the wall of pressure vessel 3 for the purpose of indicating the heat radiation therein which, in combination with the value for the residual pressure in the pressure vessel, will give a value which can be converted in a manner known per se to indicate the temperature of the work piece at any given time. The weight of lid 10 and the pressure differential pressing the lid against the packing will serve for hermetic sealing and quick evacuation of the pressure vessel.

Conduit 14 connecting pump 4 with pressure vessel 3 may also communicate in per se known and not illustrated manner with several additional pressure vessels 3, whereby each of the pressure vessels will require only about two minutes for being evacuated down to a residual pressure of about 15 mm. mercury.

After such evacuation, the further cooling of the work pieces in the respective pressure vessels does not require any supervision and generally will require several hours, depending on the shape and primarily the mass of the respective work piece.

Preferably, as a further safeguard, there is also provided a valve 14 which may be actuated in conventional magneto-electrical manner.

The specific electronic control devices utilized in connection with operating the arrangement of FIG. 1 are per se conventional and not illustrated. They operate inexpensively and reliably.

The pressure vessel 3 as illustrated has a capacity of 280 liters and pump 4 a capacity of 60 cubic meters per hour. When it is desired to evacuate the pressure vessel further, down to a residual pressure of about 2 mm. mercury, it is still possible with one pump 4 to operate six pressure vessels 3 without experiencing any difficulties.

It is also possible to arrange thermometer 13 so that the same will be in direct contact with the work pieces within the pressure vessel. This may be accomplished by resiliently mounting thermometer 13 and will operate

satisfactorily since no quick movements of the work pieces will take place.

The periods of time during which work pieces should be allowed to cool by heat radiation while located in the evacuated pressure vessel will depend primarily on the weight or mass of the work piece and differ only very little with respect to the specific composition or shape thereof.

Generally, it has been found that the desired results, i.e. a cooling to below 200 and preferably to about 150° C., will be achieved with work pieces of 5 kilograms in about 2½ hours, weighing 8 kilograms in about 3½ hours, weighing 18 kilograms in about 6½ hours and weighing 25 kilograms in about 9 hours.

After such cooling times, the work piece surface was found to have cooled down by heat radiation to about 150° C. and removal of the work piece from the pressure vessel and exposure of the work piece to the ambient atmosphere was then possible without any risk of damage to the surface of the work piece or of the formation of tension cracks.

In theory, the interior dimensions of the pressure vessel are of no consequence since heat radiation emanates radially from the work piece in all directions. True radiation will occur as long as the surroundings are colder than the work piece. For this reason, it is desirable to use pressure vessels which are provided, in their walls, with conventional water cooling. In this manner, the cooling period may be reduced to about one-fifth of that achieved without water cooling, particularly in cases in which the volume of the work piece or work pieces is substantial relative to the inner volume of the pressure vessel 3. The temperature of the pressure vessel walls may be maintained by water cooling at about 20° C. so that initially a temperature differential of nearly 500° C. will exist between the temperature of the work piece and the temperature of the walls of the pressure vessel. Without such water cooling, the walls of the pressure vessels would warm up and would produce heat radiation in the direction towards the work piece so that the temperature differential would be less than 50% of that achieved with water cooling. Quite obviously, the temperatures of the work piece, as well as of the vessel walls, change during the cooling and the foregoing figures are given only by way of a rather extreme example. For the cooling of very expensive work pieces, or work pieces which are particularly sensitive to cracking, water cooling is reduced or eliminated and thereby the cooling period is prolonged, generally up to about 10 hours. In this case, only time but no additional work or energy is expended.

The work pieces 6 may consist, for instance, of sintered bodies of chromium-nickel steel or of highly alloyed tools of chromium steel or SS-steel or may be produced of other alloys in a great variety of sizes and shapes, and in all these cases, even after a useful life span of the nitrided work pieces of several months, no tension cracks were observed. Particularly tools for warm working such as pressure casting molds for casting light or heavy metals can be treated successfully in accordance with the present invention, whereby due to the fault-free surfaces adherence between tool and mold will not take place. It was interesting to note thereby that the corrosion layer formed on the surface of the thus-treated tools could be eliminated in an even more simple manner than corrosion layers formed on work pieces which were cooled in conventional manner by quenching in oil. Since water quenched tools have an even greater surface roughness, it was found that, notwithstanding the prolonged cooling periods, the work pieces which were cooled in accordance with the present invention had optimum surface characteristics.

It is well known that the surfaces of nitrided work pieces may be improved, i.e. may be smoothed by being subjected for a short period of time to dull lapping with

## 11

silicon carbide having a particle size passing through 800 mesh. In this manner, the residual roughness can be reduced to between 1 and 2 microns. If in addition a polishing lapping with glass pearls is carried out, then the thus-treated surface obtains a silken smooth appearance, whereby only fractions of 1 micron of the surface layer are removed.

It was found that by proceeding in accordance with the present invention, the work pieces 6 which are removed from pressure vessel 3 had in all cases a thin grey corrosion layer of surprisingly low stability. It was found that the dull lapping with hard silicon carbides was not necessary and that the polishing lapping with a dispersion of glass pearls in water or the like fully suffices. Thereby, the hardness-providing compound surface zone remains completely undisturbed. Practical experience has shown that drawing tools which are exposed to a great degree of stress when hardened in accordance with the present invention, possessed a substantially prolonged useful life span. Tools hardened in accordance with the present invention and then used for the heat deformation of light metals could be used without any subsequent surface treatment, after washing off of the salt layer and removing residual impurities with a soft brass brush.

It is a further advantage of the present method as compared with quenching in oil that the washing of the nitrided work pieces which were treated in accordance with the present invention can be carried out simply with cold water.

It is particularly important and significant that by proceeding in accordance with the present invention only a very thin corrosion layer is obtained which layer, as has been described, can be easily removed without damaging the important thin, hard compound layer of, for instance, iron carbides and iron nitrides.

In the case of work pieces which were subjected to conventional nitriding and cooling, very uneven corrosion layers are formed, the structure of which depends to a considerable extent on the structure and composition of the alloy and which corrosion layers themselves are subject to heat stresses. For this reason, such corrosion layers formed in conventional processes may partially break off during the cooling of the work piece and thereby an extremely rough and difficultly workable surface is formed. These disadvantages are not experienced when proceeding in accordance with the present invention.

Referring now to FIG. 2, the same shows by way of example an extrusion die 20 which may be treated in accordance with the present invention. The extrusion opening 21 which is cut into die 20 serves for the extruding of aluminum rods which are used as building elements for windows, doors and the like. The complicated cross-sectional configuration of the extrusion opening frequently led to tension cracks and the surface of extruded aluminum alloy rods which were formed by extrusion through hardened dies of the type of die 20 frequently show fine longitudinal grooves, due to the fact that it is not possible to effectively work the hardened surfaces defining the extrusion orifice 21. However, by hardening such dies in accordance with the present invention, no tension cracks occurred, the hardly accessible inner surface areas could be easily cleaned and were found then to be practically as smooth as prior to the hardening treatment.

FIG. 3 illustrates as a further example of a work piece a forging die which combined with a similar die serves for producing valve bodies and which also has been hardened in accordance with the present invention, in an arrangement as illustrated in FIG. 1.

The surfaces of the hardened work pieces were of the desired smoothness and particularly the critical areas 31 as well as areas 32 remained of accurate size even upon prolonged use under high stress no tension cracks occurred.

Similar results were obtained, for instance, by nitriding the crankshaft illustrated in FIG. 4 wherein particularly hardening of bearings 41, 41', 41" and of crankshaft

## 12

bearings 43, 43' and 44 and 44' are of importance, although simultaneously also main shaft 42 and pinion 45 were subjected to nitriding and hardening.

As pointed out further above, the cooling method of the present invention may also be used for the cooling of work pieces, especially work pieces formed of alloyed steel, which were subjected to nitriding in a hot nitrogen atmosphere and which thereafter may be introduced without substantial delay but in contact with the ambient atmosphere, into pressure vessel 3 and therein cooled, as described above, by heat radiation while maintained at a residual pressure of for instance 5 mm. mercury.

The following examples are given as illustrative only without, however, limiting the invention to the specific details of the examples.

## Example 1

An extrusion die as illustrated in FIG. 2 is to be nitrided.

The die consists of alloyed steel containing 0.4% carbon, 5% chromium, 1.5% molybdenum and 1% vanadium, and has a weight of 2.85 kg.

The diameter of the die is 13.8 cm. and the extrusion opening 21 is formed with an accuracy of  $\pm 0.15$  mm. The surface roughness of the inner faces of the extrusion opening does not exceed 2 microns. The radii in the corners or edges of the extrusion opening 21 are smaller than 0.5 mm.

This blank has been warm hardened. Its dimensions are sufficiently accurate and the surfaces defining the extrusion opening 21 are highly smooth. There are no cracks in the edge portions of the extrusion opening and it is therefore possible to use die 20 for extruding therethrough aluminum alloys into a shape corresponding to that of extrusion opening 21.

However, the wear and tear on die 20 is very high, particularly if relatively hard aluminum-silicon-magnesium alloys are to be extruded. Even by taking greatest care with respect to extrusion temperature, extrusion speed and lubricating agents, the useful lifespan of die 20 is rather limited so that the costs of providing the die will amount to about 6% of the total cost of the aluminum bodies extruded therethrough, since aluminum alloy particles adhere on the die 20.

However, if such die is hardened in a nitriding bath the useful lifespan of the die can be increased four to sixfold without impairing of quality of the extruded rods so that the die costs will then amount to not much more than 1% of the total costs of the extruded rods. However, this saving is substantially lost because the costs of conventional nitriding of the die increase the costs thereof by 100%.

The high cost of nitriding are due to the following:

The nitriding bath consists of a molten salt mixture containing cyanides and cyanates and having a temperature of 570° C. Such salt mixture is commercially available under the trademark "Tenifer." Die 20 remains in the molten salt bath for 80 minutes and thereby, due to diffusion, an alloy or compound zone is formed having a thickness of about 20 microns and consisting essentially of iron carbide and iron nitride.

This alloy zone is very hard but also very thin. The hardened die is removed from the salt bath at a temperature of 570° C. It has to be quenched or at least quickly cooled since otherwise the surfaces would corrode.

Cooling in an ambient atmosphere causes the formation of irregular corrosion layers and a roughness of about 5 microns. Consequently, it is necessary to work the thus-roughened surfaces. This is difficult and expensive because the surfaces have now been nitrided. Furthermore, such working removes a substantial portion of the hard nitride layer. In addition, such cooling in ambient atmosphere is connected with the danger of dimensional distortion due to interior heat tensions. Further working by grinding is extremely difficult and causes removal of another portion of the hard layer.

Consequently, by proceeding in this manner, the desired dimensional correctness of the die can no longer be maintained.

Cooling by quenching in water will give a better surface layer, however, the dimensional distortion will be excessively large. Furthermore, by quenching in water, more than 20% of the dies are ruined by heat tension cracks. Such cracks cause immediately or after a very short period of time breaking of the die 20. Dies such as die 20 with cracks formed therein, which cracks primarily occur in the edges of the extrusion opening 21, are not usable. Such cracks cannot be subsequently welded since the material contains N. Obviously, it is not possible to extrude rods of the desired cross-sectional shape by utilizing a die which has a visible crack since the markings of the crack will be seen at the outer face of the extruded rod and furthermore since the zone of the die in which the crack is located will quickly break so that the entire extrusion device will have to be stopped. All of these disadvantages result in considerable additional cost due to frequent interruptions of the extrusion operation as well as due to loss of the labor involved in the preparation of the unhardened die 20.

Consequently, the only practical method appears to be the quenching in an oil bath. However, it has been found that in the case of dies such as die 20 of FIG. 2, a waste of between 11 and 12% will be caused due to heat cracks which sometimes are immediately apparent and sometimes are found after very short use of the die. It is not possible to determine with certainty by visual inspection whether or not the hardened die 20 has fine cracks, within the surfaces defining the extrusion opening 21 and even if no actual crack has been formed, it is possible that the die has been dimensionally distorted by heat tensions so that further working would be required.

For all these reasons, it was possible by quenching the nitrided die in an oil bath to prolong the useful lifespan of the die about six times, however, the production costs per useful hardened die were about 100% higher than for the unhardened die.

By proceeding in accordance with the present invention, it was possible to avoid this increase in the costs of the die. It was found that by nitriding the die in a molten salt bath and then cooling as described above in accordance with the present invention, practically no waste material was formed and substantially 100% of the treated dies could be operated for the above indicated prolonged period of time.

This was accomplished as follows:

The dies 20 were hardened as before for 80 minutes at 570° C. in a nitriding salt bath and then removed therefrom. The thus-hardened dies were simply transported through the ambient atmosphere into the pressure vessel 3 of FIG. 1 and hung into the same. The time required for the removal of the hardened die from the salt bath to closing lid 10 of pressure vessel 3 after insertion of the die into the pressure vessel amounted to about 30 seconds and the temperature drop during this period equaled about 1.5° C. per second or a total of about 45° C.

Immediately after closing lid 10, vacuum pump 4 was actuated and thereby the drop in temperature by heat conduction and convection was quickly effectively reduced. After operating the pump for 2 minutes the residual pressure in the pressure vessel amounted to 15 mm. mercury. During this period of 2 minutes, the temperature loss at the surface of the hardened work piece was reduced from 1.5° C. to only about 0.035° C. per second so that the average temperature loss during these two minutes amounted to 0.23° C. per second.

Thus, upon establishing a residual pressure of 50 mm. mercury the temperature of die 20 was still higher than 480° C.

Further cooling took place nearly exclusively by heat radiation.

After 2 hours and 15 minutes, pressure vessel 3 was

opened and it was found that the die 20 located therein had a temperature of less than 200° C. (estimated). The first measurement was made 12 seconds after opening of the lid 10 and at that time the surface temperature of the die, probably due to contact with the air entering the pressure vessel, was less than 150° C.

It is of course also possible to reduce ambient pressure by the introduction of heated air, however, this has been found to be unnecessary for a variety of reasons.

First of all, obviously cracks were not formed during the initial drop in the temperature from about 570° C. to 480° C. and during this period also no dimensional distortion of any significance did occur. Furthermore, during these first 30 seconds plus maximum 2 minutes, i.e. until a residual pressure of 15 mm. mercury had been established, no appreciable corrosion took place at the still liquid salt-covered surface of the die, notwithstanding the contact with the surrounding ambient atmosphere and the oxygen content of the latter.

Secondly, the critical temperature range of from 480° C. to below 200° C. was passed so slowly (within 2½ hours) that obviously cracks could not be formed by such slow cooling. Possibly, initial heat tensions were equalized during this period and, most important, due to the practically complete lack of an atmosphere, no further corrosion took place.

Finally, the somewhat quicker cooling from below 200° C. down towards ambient temperature which occurred upon removal of the die, was sufficiently mild or slow so that no cracks could be formed and, due to the relatively low initial temperature, i.e. below 200° C., no visible enlargement of the corrosion layer took place. The existing corrosion layer was of gray color, as usual, however, surprisingly, it was very easily removable. Very significant was the high degree of smoothness of the surface which had a roughness of only between about 1 and 2 microns. It was possible to use the thus-cooled die without any further treatment for the extrusion therethrough of profiled rods of aluminum-silicon-magnesium alloys. It was found that only the first 30–40 cm. of the extruded rod were of somewhat lesser smoothness, but after extruding such relatively small length, the corrosion layer at the surface of extrusion opening 21, i.e. the inner surface of die 20 was completely removed.

The result of proceeding in this manner was a cost reduction of more than 50% as compared with previously produced hardened dies and fault-free production of high quality hardened dies. The total die costs amounted to less than 1% of the total costs of producing the extruded aluminum rods.

#### Example 2

The work piece illustrated in FIG. 3 of the drawing, i.e., a forging die, was subjected to the process of the present invention.

The weight of die 30 was 1.65 kg. and the die was formed of a chromium-molybdenum steel of the type H13.

Hardening of the die was carried out as described in Example 1 by immersing the die in the nitriding salt bath maintained at 570° C.

It was found that generally a cooling period of 2 hours will suffice for work pieces weighing less than 3 kg., unless so many individual work pieces are introduced into one pressure vessel 3 that due to the total mass of cooling metal therein the cooling period was prolonged.

The pressure vessel 3 was provided with water cooling in its cylindrical wall. Tap water was passed in contact with the wall of the pressure vessel so that the outer temperature of the wall remained below ambient temperature and the spent cooling water was heated to a temperature of only between about 20 and 30° C.

While generally proceeding as described in Example 1, it was found as a particular advantage in this case that

particularly no dimensional distortion occurred during the cooling. Consequently, two exactly pre-fashioned drop forging dies 30 will have an excellent fit even without working the surfaces of the dies after the hardening and cooling of the same. By using dies of the type illustrated in FIG. 3 for producing valve bodies, coaxial products are obtained practically free of fins so that only little further working of the pressed product produced in such die will be required. The surface roughness of the cooled die was only between 1 and 2 microns and the thin gray corrosion layer which was formed similar to the layer formed according to Example 1, is in this case preferably removed by lapping, preferably wet lapping which may be carried out by spraying a dilute aqueous soap solution against the surfaces 31. It can also be carried out by spraying a dispersion of very small glass spheres in water. These various lapping methods are well known to those skilled in the art.

Again it was noted that crack formation was completely absent, the hard nitrided layer was completely maintained since no material-removing further working was required. Consequently, the useful lifespan of the drop forge dies was prolonged and thus also the number of valve bodies that could be produced with one pair of the dies.

### Example 3

The crank shaft illustrated in FIG. 4 was subjected to nitriding and cooling in accordance with the present invention. Before nitriding the forged shaft was warm hardened.

The crank shaft was produced by drop forging of the alloy identified as 42CrMo4, and weighed 11.2 kg.

Hardening was carried out as described in Example 1 at a temperature of 570° C. The residence time of the crank shaft in the salt bath was 90 minutes and it was found that the thickness of the hard compound surface zone was more than 20 microns.

Removal of the crank shaft from the salt bath and introduction into the pressure vessel 3 required 30 seconds and two minutes later a residual pressure of 15 mm. mercury was reached in pressure vessel 3.

Due to the greater size of crank shaft 40 as compared with the work pieces described in Examples 1 and 2, the extent of cooling during transfer of the work piece from the bath into the pressure vessel was somewhat less and amounted only to 35° C. and to the point at which the residual pressure of 15 mm. mercury was reached only to about 60° C. The residence time of the crank shaft in evacuated pressure vessel 3 was 4 hours and upon subsequent removal the temperature of the crank shaft was 160° C.

No measurable dimensional distortion was found and therefore it was also not necessary to carry out any further working. It was also not necessary to subsequently grind any of the bearing faces. The corrosion layer could be sufficiently removed by spraying with soap solution. The surface roughness was only 1 micron. The thus-cooled crank shaft could be immediately mounted without requiring any further treatment.

Without further analysis, the foregoing will so fully reveal the gist of the present invention that others can by applying current knowledge readily adapt it for various applications without omitting features that, from the standpoint of prior art, fairly constitute essential characteristics of the generic or specific aspects of this invention and, therefore, such adaptations should and are intended to be comprehended within the meaning and range of equivalence of the following claims.

What is claimed as new and desired to be protected by Letters Patent is set forth in the appended claims:

1. A method of nitriding a ferrous workpiece, comprising the steps of immersing said workpiece in a molten nitriding salt bath at a temperature significantly above about 500° C.; conveying the thus nitrided hot workpiece through the ambient atmosphere into a pressure vessel at such speed that the temperature of said hot nitrided workpiece will drop during said conveying by not more than about 100° C.; evacuating said pressure vessel promptly after introduction of said workpiece into the same to a residual pressure of up to about 20 mm. Hg; and allowing said workpiece to cool by heat radiation while located in the thus evacuated zone and simultaneously cooling said pressure vessel to counteract the heating 25 of the walls of the pressure vessel during cooling of the workpiece.

2. A method as defined in claim 1, wherein said hot workpiece is conveyed from said nitriding into said evacuable zone at such speed that the temperature of 30 said hot nitrided workpiece will drop during said conveying by less than the difference between said nitriding temperature and about 500° C. so that said workpiece will be introduced into said pressure vessel at a temperature of at least about 500° C.

3. A method as defined in claim 1, wherein said metallic workpiece consists essentially of steel.

4. A method as defined in a claim 1, wherein said pressure vessel is evacuated to a residual pressure of between about 2 and 20 mm. Hg.

5. A method as defined in claim 1, wherein said pressure vessel is evacuated to a residual pressure of up to about 2 mm. Hg.

6. A method as defined in claim 1, wherein said cooling of said workpiece in said pressure vessel by heat radiation is continued at least until the temperature of said workpiece has been lowered to about 150° C.

7. A method as defined in claim 1, wherein said nitriding temperature is about 570° C.

50

### References Cited

#### UNITED STATES PATENTS

|              |         |         |       |           |
|--------------|---------|---------|-------|-----------|
| 1,644,828    | 10/1927 | Guibert | ----- | 148—16.7  |
| 1,953,647    | 4/1934  | Darrah  | ----- | 148—15.5  |
| 55 1,961,520 | 6/1934  | Malcolm | ----- | 148—15.5  |
| 2,041,769    | 5/1936  | Larkin  | ----- | 148—15.5X |
| 2,916,409    | 12/1959 | Bucek   | ----- | 148—16.6X |

CHARLES N. LOVELL, Primary Examiner